

## [54] DURABLE FIRE RETARDANT TEXTILE MATERIALS BY ANHYDROUS SOLVENT FINISHING PROCESS

[75] Inventor: James M. Thompson, Salisbury, N.C.

[73] Assignee: Proctor Chemical Company, Inc., Salisbury, N.C.

[22] Filed: Sept. 25, 1972

[21] Appl. No.: 292,145

[52] U.S. Cl..... 117/136, 117/137, 117/139.4

[51] Int. Cl..... C09d 5/18

[58] Field of Search..... 117/136, 137, 139.4; 106/15 FP; 252/8.1

## [56] References Cited

## UNITED STATES PATENTS

|           |         |                   |             |
|-----------|---------|-------------------|-------------|
| 2,385,766 | 9/1945  | Thurston.....     | 117/135.5   |
| 2,749,257 | 6/1956  | Knup et al.....   | 117/139.4 X |
| 2,887,409 | 5/1959  | Van Loo.....      | 117/139.4   |
| 3,091,612 | 5/1963  | Stephens.....     | 117/132 B X |
| 3,323,939 | 6/1967  | Van Loo.....      | 117/139.4 X |
| 3,434,870 | 3/1969  | Touey et al.....  | 117/139.4 X |
| 3,471,318 | 10/1969 | Redfarn.....      | 106/15 FP X |
| 3,615,743 | 10/1971 | Theuer.....       | 106/15 FP X |
| 3,658,575 | 4/1972  | Tabor et al.....  | 117/136 X   |
| 3,668,302 | 6/1972  | Boland et al..... | 117/136 X   |
| 3,690,941 | 9/1972  | Reuter et al..... | 252/8.1 X   |
| 3,695,926 | 10/1972 | Scarborough.....  | 117/136     |
| 3,729,340 | 4/1973  | Powell .....      | 117/136     |

3,746,572 7/1973 Weil et al. .... 117/136

## FOREIGN PATENTS OR APPLICATIONS

|           |        |                    |           |
|-----------|--------|--------------------|-----------|
| 747,014   | 3/1956 | Great Britain..... | 117/136   |
| 1,204,163 | 9/1970 | Great Britain..... | 117/139.4 |
| 1,241,926 | 8/1971 | Great Britain..... | 117/139.4 |

## OTHER PUBLICATIONS

"Chemical Abstracts" by American Chemical Society  
 Volume 47, Number 13, July 10, 1953, pages  
 7230-7231.

Primary Examiner—William D. Martin

Assistant Examiner—Theodore G. Davis

Attorney, Agent, or Firm—Kemon, Palmer & Estabrook

## [57] ABSTRACT

Anhydrous solvent finishing processes to impart durable fire retardant properties to textile materials, e.g., flat goods or finished garments, made of cellulosic fiber, polyester fiber or fiber blends of such fibers with other fibers, involve (a) impregnating textile material with an anhydrous mixture of tris-polyhaloalkyl phosphate, nitrogenous film forming binder resin, organic solvent and organic aminoplast cross-linking catalyst, (b) removing solvent, and (c) heat curing at about 120° to 200°C. The anhydrous organic solvent mixture may include soluble crease-proofing agents so that the resulting fabric acquires both durable press and fire retardant properties.

9 Claims, No Drawings

**DURABLE FIRE RETARDANT TEXTILE  
MATERIALS BY ANHYDROUS SOLVENT  
FINISHING PROCESS**

**BACKGROUND OF THE INVENTION**

1. Field of the Invention

The invention relates to the finishing of fabrics and other textile materials made of cellulosic fibers to impart durable fire retardant qualities thereto. More particularly, it concerns anhydrous solvent finishing methods for textile materials capable of creating good fire retardant ratings for the textile material that are durable to repeated launderings and, in some embodiments, simultaneously also creating durable crease resistance.

2. Description of the Prior Art

Textile articles that have fire retardant properties durable even after repeated launderings are much in demand. Federal laws require certain classes of garments to be durably fire retardant and the classes of garments to which these requirements will apply is due to expand (see "Chem. & Eng. News", 50 (29), July 17, 1972, p.22).

Fire retardant properties in textile materials can be obtained in a variety of ways. However, many of the known methods do not create fabrics in which the fire-retardancy is capable of withstanding repeated launderings. Cotton fabrics, for example, are relatively easy to treat with ammonium phosphate, ammonium sulfamate and mixtures of borax and boric acid. Unfortunately, such treatment does not impart durable fire-retardancy.

Extensive use has been made of phosphorus and halogen containing compounds to impart fire retardant properties to textiles and other substrates. In characterizing the ultimate fire-retardancy of such compounds, a convenient notation known as "Fire Retardant Index" may be utilized. The index of any particular material is calculated on a weight basis utilizing the following equation:

$$FRI = 10 (P\%) + 2(Br\%) + (Cl\%) + 2(N\%)$$

For example, a compound containing 5%, by weight, phosphorus and 50%, by weight, bromine would exhibit as FRI of 150. It has been determined that for general industrial applications, an FRI of at least about 60 is required to impart satisfactory fire retardance. FRI values of at least about 80 are usually required for use with cellulosic substrates.

One type of compound widely used to impart fire-retardancy is tris-haloalkyl phosphates. They have been used combined with an organic resin binder and coated on textiles (see U.S. Pat. No. 3,471,318), mixed with phenolic resins to impregnate cellulosic sheets in forming structural laminated panels (see U.S. Pat. No. 3,549,479) and used as an ingredient in aerosol sprays used to fire-proof textiles or other substrates (see U.S. Pat. No. 3,607,745). Bis-haloalkyl phosphates have also been used, e.g., the ammonium salt of bis-(2,3-dibromopropyl) phosphate (see U.S. Pat. No. 3,660,582) and the amides of brominated dialkylene phosphates (see U.S. Pat. No. 2,574,518). A further discussion of the use of the haloalkyl phosphates for fire-proofing can be found in Little, "Flameproofing Textile Fabrics", Reinhold Publishing Corp., New York (1947).

Difficulties have been encountered in use of haloalkyl phosphates as disclosed in the prior art. One diffi-

culty relates to their limited hydrolytic stability. This may be encountered in the utilization of the phosphate on substrates with the result that fire retardant groups are either readily leached from the substrate or converted on the substrate to non-fire retardant alkaline earth phosphate salts during wet launderings.

In order to overcome the problems of the phosphates, phosphonates have been used instead (see U.S. pat. No. 2,803,562 and 3,325,563). Polymerizable phosphonates have been used to impregnate fabrics and form in situ fire retardant polymers, e.g., wool treated with bis-chloroethyl vinyl phosphonate (see U.S. Pat. No. 3,669,610).

While the phosphonates exhibit greater hydrolytic stability, they are more costly, and at high concentrations required for fire-retardancy, it is difficult to utilize these phosphonates in the treatment of substrates for fire retardance. Hence, there is a need for new methods to use fire-proofing haloalkyl phosphates while avoiding the hydrolytic instability problem so that treated products can be obtained that will retain good fire-retardancy even after repeated wet launderings.

**OBJECTS**

25 A principle object of the present invention is the provision of new methods for durably increasing the fire-retardancy of textile products.

Further objects include the provision of:

1. New compositions for treatment of fabrics to improve their fire retardance properties.

2. New textile products having fire retardance that is durable even to repeated wet launderings of the products.

3. New methods for rendering fabrics both durably fire retardant and durably crease resistant, i.e., for producing durable press fabrics having durable fire-retardancy.

4. New anhydrous solution systems and methods for finishing of textile materials to render them durably fire retardant.

Other objects and further scope of applicability of the present invention will become apparent from the detailed description given hereinafter; it should be understood, however, that the detailed description, while indicating preferred embodiments of the invention, is given by way of illustration only, since various changes and modifications within the spirit and scope of the invention will become apparent to those skilled in the art from this detailed description. It should also be understood the foregoing abstract of the disclosure is for the purpose of providing a non-legal brief statement to serve as a searching-scanning tool for scientists, engineers and researchers and is not intended to limit the scope of the invention as disclosed herein nor is it intended it should be used in interpreting or in any way limiting the scope or fair meaning of the appended claims.

**SUMMARY OF THE INVENTION**

60 These objects are accomplished according to the present invention by application to a textile product of an anhydrous organic solvent solution containing (a) polyhaloalkyl phosphate as hereinafter defined and (b) nitrogenous film forming synergistic binder resin as hereinafter defined, evaporation of volatile solvent from the solution containing textile product and heat curing of the reagents retained in the textile product,

preferably promoted by the presence of (c) an aminoplast curing catalyst, to fix the reagents (a) and (b) upon the fibers of the textile product.

Advantageously, the solution applied to the textile product will contain (d) a nitrogenous crease-proofing agent as hereinafter defined and the solvent-depleted textile material will be subject to a moisture regain step before the heat curing step to provide between about 8 to 15% moisture in cellulosic fiber content of the textile product.

Anhydrous solutions useful in the invention will contain in a volatile organic solvent 5-50% of ingredient (a) and 2-20% of ingredient (b). If used, ingredient (c) will be present in 0.1-5% and ingredient (d) in 5-20%. All such ingredients may consist of a mixture of several reagents.

Application of the anhydrous solution, e.g., by impregnation, to the textile product is conducted to provide in the fabric such quantity of solution that the weight ratio of ingredient (a) to the dry weight of the fabric will be between about 1: 20 and 1: 2. Additionally, the percent add on by weight to the textile product of ingredient (b) will preferably be between about 2 to 15%.

Stated briefly, processes for the production of durable fire retardant textile materials in accordance with the invention involve the following steps:

A. providing a substantially anhydrous solution comprising:

- a. polyhaloalkyl phosphate
- b. nitrogenous film forming binder resin
- c. organic solvent having a boiling point below about 200°C.

B. applying said anhydrous solution to a textile product in such quantity that the weight ratio of said ingredient (a) based on the dry weight of the textile product is between 1: 20 and 1: 2.

C. evaporating substantially all volatile organic solvent from the textile product resulting from step B, and

D. heating the solvent freed textile product to a temperature of between about 120°C. to 200°C. for a time between about 1 and 30 minutes to cure and fix the ingredients retained in the textile product upon said product.

Preferably, ingredient (a) is tris-2,3-dibromopropyl phosphate and ingredient (b) is an organic solvent soluble melamine or triazine aminoplast resin, especially methoxy methyl melamine or butoxymethyl benzo quanomine.

As the organic solvent of the anhydrous systems used in accordance with the invention, halogenated hydrocarbons are advantageous not only because they are highly effective in the operations but also from a safety viewpoint if non-flammable halogenated hydrocarbons are used. However, the new methods are effective with the use of other water-immiscible organic solvents including hydrocarbons, esters and ethers. The anhydrous solvent may contain up to about 10% of an aliphatic alcohol or an alkoxyalkane to improve the solubility of the methylolated carbamate used in the anhydrous system as the durable press producing agent.

As to the catalyst used to promote curing of the nitrogenous film forming binder resin, a variety of organic solvent soluble compounds having cross-linking catalytic effect on aminoplasts are known and can be used. Advantageously, from among these, a catalyst will be selected which does not adversely affect fabric

strength, color or other desired qualities. By way of example, p-toluene sulfonyl chloride has been found particularly useful. Preferred catalysts are those selected from the group consisting of haloaryllactones, halides and monocyclic aryl sulfonyl halides.

A mild alkaline afterwash of conventional type may be employed to improve the aesthetics of the final product. Fabric strength degradation by the new processes is less than 15% of the untreated fabric strength.

10 Success of the invention is, in part, due to the discovery that durable press properties can be produced in cellulosic textile materials simultaneously with fire retardant properties using the same anhydrous solvent systems as outlined above relative to the durable press agent. Methylolated carbamates constitute a preferred type of crease-proofing agent for use in these new textile treatments as disclosed hereinafter and also in co-pending application Ser. No. 215,626, filed Jan. 5, 1972, now U.S. Pat. No. 3,834,871, the disclosure of 15 which is incorporated herein by reference.

#### DESCRIPTION OF PREFERRED EMBODIMENT

The following details of operations in accordance with the invention and reported data illustrate the further principles of practice of the invention to those skilled in the art. In these examples and through the remaining specification and claims, all parts and percentages are by weight unless otherwise specified.

##### Example 1

A clear solution was made by stirring together the following ingredients in the parts specified:

|                                    |          |
|------------------------------------|----------|
| tris-(2,3-dibromopropyl) phosphate | 20 parts |
| tri-(methoxy methyl) melamine      | 5 parts  |
| 1,1,1-trichloroethane              | 75 parts |

The resulting straw colored solution was used to impregnate 100% viscose rayon fabric to a wet pickup of 70%. The fabric was allowed to air dry at room temperature (20°-25°C.) for 10 minutes and was then given a hot air cure of 1 minute at 150°C.

Samples of the treated rayon fabric were subjected to (DOC-FF-371) (vertical char method) which gave a char length value of four three-fourth inch with no after flame or after glow. The fabric was then subjected to successive launderings (AATCC Test 124) and was checked for fire retardant properties after 5 and 10 launderings. All such tests gave char lengths of 7 inches or less with no after glow and no after flame.

##### Example 2

Using the anhydrous solution of Example 1, 100% cotton broadcloth fabric was impregnated to a wet pickup of 80%. The fabric was allowed to air dry 10 minutes and then given a hot air cure of one minute at 150°C. The resulting fabric gave a value of 5 inch char length on DOC-FF-371 Test (vertical char) with no after flame or after glow. As in Example 1, 5 and 10 launderings (AATCC Test No. 124) gave char lengths of 7 inch or less with no after glow or after flame.

##### Example 3

Using the anhydrous solution of Example 1, a 50% polyester/50% cotton muslin sheeting fabric was impregnated to a wet pickup of 65%. The fabric was run over low pressure steam drums continuously to effect

solvent removal and recovery. After this, the fabric was given a hot air cure at 165°C. for 1 minute. When tested according to DOC-FF-371 Test, the char length was five one-half inch. Following 5 and 10 launderings (AATCC Test No. 124) gave char length values of less than 7 inch. There was no after glow or after flame in any of the tests.

#### Example 4

A clear solution was made of the following ingredients:

|                                         |           |
|-----------------------------------------|-----------|
| N,N-dimethylol-2-methoxyethyl carbamate | 125 parts |
| p-toluene sulfonyl chloride             | 10 parts  |
| tris-(2,3-dibromopropyl) phosphate      | 250 parts |
| methoxy methyl melamine                 | 50 parts  |
| 1,1,1-trichloroethane                   | 565 parts |

A 100% cotton broadcloth was impregnated with the solution and then pad-squeezed to a wet pickup of 80%. The fabric was air dried at room temperature for 10 minutes and then lightly steamed to produce a moisture regain of 10-15%. Finally, the fabric was cured for 1 minute at 160°-165°C. The ambient conditioned fabric when tested produced the following data:

Crease Recovery (AATC No. 66—Recovery Angle Method) warp and filling) = 278°

Durable Press Rating (AATC No. 124 — Durable Press Replica) after one home laundering = 4.0

After 50 launderings = 3.8-4.0

Vertical Char (DOC-FF-371) = 4.5 inch (one laundering) no flame or after flow

Vertical Char = 7-8 inch (10 launderings) no flame or after glow

#### Example 5

A clear solution was made of the following ingredients:

|                                         |           |
|-----------------------------------------|-----------|
| N,N-dimethylol-2-methoxyethyl carbamate | 150 parts |
| p-toluene sulfonyl chloride             | 10 parts  |
| tris-(2,3-dibromopropyl) phosphate      | 200 parts |
| methoxy methyl melamine                 | 50 parts  |
| 1,1,1-trichloroethane                   | 615 parts |

A 100% viscose rayon prepared fabric impregnated with the solution to a wet pickup of 70%. The fabric was dried by solvent evaporation for 10 minutes at room temperature and then lightly steamed to a moisture regain of 8-15%. Finally, the fabric was hot air cured for 1 minute at 160°-165°C. The ambient conditioned fabric when tested produced the following data:

|                            |                                                    |
|----------------------------|----------------------------------------------------|
| Crease Recovery            | = 265°                                             |
| Durable Press Rating       | = 3.8 (one laundering)                             |
| Durable Press Rating       | = 3.5 (50 launderings)                             |
| Vertical Char (DOC-FF-371) | = 4.5" (one laundering)<br>no flame or after glow  |
| Vertical Char (DOC-FF-371) | = 7.0 (10 launderings -<br>no flame or after glow) |

#### Example 6

As in Example 1, a clear solution was made of the following ingredients:

|   |                                         |           |
|---|-----------------------------------------|-----------|
| 5 | N,N-dimethylol-2-methoxyethyl carbamate | 125 parts |
|   | p-toluene sulfonyl chloride             | 10 parts  |
|   | tris-(2,3-dibromopropyl) phosphate      | 350 parts |
|   | methoxy methyl melamine                 | 50 parts  |
|   | 1,1,1-trichloroethane                   | 465 parts |

A 50/50 polyester/cotton prepared sheeting fabric (percale) was impregnated with the solution to a wet pickup of 60% and then allowed to dry at room temperature by solvent evaporation. The dry fabric was steamed to a moisture regain of 8-15% based upon the weight of the cellulosic component of the fabric. Finally, the fabric was hot air oven cured for 1 minute at 160°-165°C. The ambient conditioned fabric when tested produced the following data:

|    |                            |                         |
|----|----------------------------|-------------------------|
| 20 | Crease Recovery            | = 285°                  |
|    | Durable Press Rating       | = 4.5 (one laundering)  |
|    | Durable Press Rating       | = 4.5 (30 launderings)  |
|    | Vertical Char (DOC-FF-371) | = 5.5" (one laundering) |
|    | Vertical Char (DOC-FF-371) | = 8-9" (10 launderings) |

#### Example 7

A clear solution was prepared by stirring together the following ingredients in the parts specified:

|    |                                    |           |
|----|------------------------------------|-----------|
| 30 | tris-(2,3 dibromopropyl) phosphate | 200 parts |
|    | butoxy methyl urea formaldehyde    | 50 parts  |
|    | perchloroethylene                  | 750 parts |

The resultant straw colored solution was used to impregnate a 100% cotton twill fabric to a wet pickup of 100%. The fabric was allowed to air dry at room temperature (20°-25°C.) for 10 minutes and was given a hot air cure of 45 seconds at 160°C.

Samples of the so treated material were tested for fire retardancy according to test method DOC-FF-371, originally, after 5 launderings and after 10 launderings. In all cases, the char lengths were less than 7 inches with no after glow or after flame.

#### Example 7

A clear solution was prepared by stirring together the following ingredients in the parts specified:

|    |                                    |                       |
|----|------------------------------------|-----------------------|
| 50 | tris-(2,3 dibromopropyl) phosphate | 200 parts             |
|    | poly-butoxy methyl pentaerythritol | 80 parts              |
|    | tetracarbamate                     | 1,1,1 trichloroethane |

The resultant solution was used to impregnate a 100% rayon drapery fabric to a wet pickup of 90%. The solvent was flashed off by high pressure steam dry cans and the fabric was given a hot air cycle of 1 minute at 160°F.

Samples of the treated fabric were tested for fire retardant properties according to test method DOC-FF-371, originally, after 5 launderings and after 10 launderings. In all cases, char lengths were less than 7 inches with no after flame or after glow.

#### Example 9

A clear solution was prepared by stirring together the following ingredients in the parts specified:

|                                    |           |
|------------------------------------|-----------|
| tris-(2,3 dibromopropyl) phosphate | 350 parts |
| tri (butoxy methyl) melamine       | 70 parts  |
| 1,1,1 trichloroethane              | 580 parts |

The resultant solution was used to impregnate a 35% polyester/65% cotton reverse blend fabric to a wet pickup of 90%. The fabric was allowed to air dry at room temperature for 10 minutes and was given a hot air cure of 1 minute at 160°C.

Samples of the treated fabric were tested for fire retardancy according to test method DOC-FF-371, originally, after 5 home washings and after 10 home washings. In all cases, char lengths were less than 7 inches with no after glow or after flame.

#### DISCUSSION OF DETAILS

The preferred haloalkyl phosphate for use with the invention is tris-(2,3-dibromopropyl) phosphate. Other tris-haloalkyl phosphates containing six to 24 carbon atoms and at least two chlorine or bromine atoms may be used including: tris-(1,2-dibromoethyl) phosphate; tris-perchloropropyl phosphate; tris-(1,2-dibromo-1,2-dichloropropyl) phosphate; tris-(1,1,1-tribromoethyl) phosphate; tris-(1,1,2,3,3,5-hexabromohexyl) phosphate; tris-perchloramyl phosphate; tris-(1,2,4,4,6,6-hexa bromooctyl) phosphate and like compounds. Advantageously, in the alkyl groups of the phosphate, the ratio halogen atoms to carbon atoms will be at least 0.5. Mixtures of two or more of the halo-alkyl phosphates may be used and, actually, the commercially available products of this type are usually a mixture of homologs.

The preferred nitrogenous film forming binder resins for use in the invention are tri-methoxymethyl melamine and butoxymethyl benzo quanamine. A variety of comparable solvent soluble nitrogenous resins are available and can be used including: dimethoxymethyl urea-formaldehyde resin, tri-methoxymethyl acetylene diureine, dibutoxymethyl-N-ethyl triazole, N,N'-ethylene-bis-dimethoxymethyl triazole, butyl ethers of methylol urea-formaldehyde polymers, butyl ethers of methylol melamine, methoxy or butoxy ethers of polymethylol penta-erythritol tetracarbamate, and the like. Mixtures of two or more such materials may be used.

Halogenated hydrocarbons having a boiling point between about 20°-200°C. and especially between about 50°-150°C., are a preferred class of anhydrous organic solvents for use in the new FR fabric treatments, e.g., 1,1,1-trichloroethane, butyl bromide, perchloroethylene, trichloroethylene, ethylene chloride, ethylene bromide, 1,1,2-trichloro-1,2,2-trifluoroethane, 1,1,1-trichloro-2,2,2-trifluoroethane, methylchloride and 1,1-dichloroethane. Other anhydrous organic solvents of similar boiling range may, however, be used including hexane, pentene-1, methyl ethyl ketone, isopropyl acetate, ethyl acetate, isopropyl ether, ethyl formate, neohexane, dioxolane, cyclohexane, cyclopentane, benzene, acetone and the like. Mixtures of two or more anhydrous organic solvents may also be used with advantage, particularly where it is desired to control evaporation or drying rate of the fabric treatment solution from the impregnated textile material.

A wide selection of aminoplast catalysts soluble in anhydrous organic solvents are available for use in the new FR treatments. Advantageously, one selects such a catalyst that will not stain or discolor the fabric, cause

excessive tendering or present safety or pollution problems. Aromatic sulfonyl halides have been found to be particularly useful, e.g., p-toluene sulfonyl chloride, benzene sulfonyl chloride, 2-chloro-4-ethylphenyl sulfonyl chloride, 2-butyl-4-ethylphenyl sulfonyl chloride, benzene sulfonyl bromide and the like. The catalyst that is used should be soluble at least to the extent of 1% in the organic solvent hereinbefore described. Advantageously,

- 5 compounds used as the catalyst are acidic or react with water to form an acidic product. Additional preferred classes of compounds to use as catalysts include halogenated aromatic lactones, e.g., chlorophthalide, bromophthalide, iodophthalide, etc. and haloimides, e.g., N-chlorosuccinimide, N-bromo- $\alpha$ ,  $\beta$ -dibromo succimide, N-chloro teraconimide, N-chlorophthalimide and the like. The amount of catalyst used will depend, in part, upon the particular carbamate reagent used, the temperature for curing and similar factors. Generally, the fabric treating solution will comprise 0.1 to 10% of the catalyst and especially 0.1 to 5%.

As illustrated by Examples 4-6, the new anhydrous treating solutions may include a nitrogenous crease-proofing agent as an active ingredient. Unique results are obtained when N,N-dimethylol alkoxy alkyl carbamates, e.g., N,N-dimethylol-2-methoxyethyl carbamate, are used for this purpose. Preferred solutions of this type will contain 5-50% of the FR phosphate, 5-20% of the binder resin, 5-20% of the crease-proofing agent, 0.1-5% catalyst, 20-80% anhydrous organic solvent and 0-20% of an auxiliary agent.

Auxiliary reagents of various types may be included in the treating solutions, advantageously in amounts between 0.1 to 20% and particularly between 0.5-15%, especially 1-10%. Such auxiliary reagents include dyes; mildew-proofing agents, sanitizing agents; softening agents; plasticizers; hand-builders and the like.

The FR treatments of the invention are usable will all varieties of cellulosic textile materials. The term "cellulosic textile material" as used herein is intended to mean any woven, knit or non-woven fabric as well as garments, bed-clothes, furniture coverings or any other textile material made in whole or in part of cellulosic fibers. Cellulosic fibers include: cotton, linen, viscose rayon, high modulus rayon (polynsic). They may be blended in yarns with synthetic fibers, e.g., nylon, polyester, polyolefin and other fibers or filaments or the textile materials may comprise mixed weaves or knits of cellulosic yarns or filaments and synthetic yarns or filaments. A particular advantage of the invention is the ability of the new operations to impart FR effects to 100% cotton textile materials without undue loss of tensile strength and abrasion resistance. In addition to cellulosic textile materials, the new methods may be applied to 100% polyester fabrics or fabrics made of blends of polyester fibers, e.g., nylon, acrylics and the like.

The anhydrous treating solutions of the invention may be applied in a variety of ways. Dipping and padding, well known in the art, can be used. Additional methods include: spraying, roller coating, float coating and the like. However, if enclosed equipment is not used, loss of solvent to the atmosphere can be costly and/or present ecological problems. Equipment is commercially available to perform the application of organic solvent treating solutions without loss of solvent

to textile material, e.g., see "Textile Industries", Oct. 1966, ps. 288-9, 291, 295, 299, 339 and 397.

The amount of solution applied will depend upon the type of fabric, e.g., wherein woven or knit and its weight, the degree of FR effect desired, the concentration of FR phosphate in the solution and similar factors. Under preferred conditions, the amount of solution relative to textile material will be selected to provide in the textile material between about 1-50%, especially 1-20%, of FR phosphate component based upon the dry weight of the cellulosic textile material. Typically, this will involve a wet pickup of treating solution between about 50-150% based upon the dry weight of the textile material.

Following the application of the anhydrous treating solution, the volatile components of the solution are removed, e.g., by evaporation. Passage of the textile material through drying ovens, through infra-red ovens or in any other suitable manner may be used. The evaporated organic solvent is removed and recovered with available solvent handling systems. As a less desirable alternative, the impregnated textile material may be permitted simply to air dry at ambient conditions.

The removal of the organic solvent from the textile material leaves a moisture and solvent depleted fabric. At this point in the new operations, the solvent depleted fabric may be exposed to water vapor to create therein a moisture regain in the cellulosic portion of the fabric of between about 8 and 15%. For 100% cotton, this will mean a total moisture regain of 8-15% while a 50% cotton/50% polyester fabric would involve a total moisture regain of 4-7.5%. Advantageously, this is accomplished by steaming of the textile material. Exposure to high humidity at room temperature or other moisture regain techniques can, however, be used. The moisture regain step is advantageous when durable press effects are also to be imparted to the fabric. More pronounced durable press effects are obtained when the moisture regain step is applied after the solvent evaporation. This also improves solvent recovery operations.

The textile material ultimately is subjected to a heat curing step to cure the resin binder and fix the FR agent upon the fabric. This heat curing may proceed immediately after the combination of solution application. Alternatively, a delay cure procedure may be used. In any event, heat curing equivalent to 1-30 minutes at 120°C. to 200°C. is used.

The embodiments of the invention in which an exclu-

sive property or right is claimed are defined as follows:

1. A process for the production of durable fire retardant textile materials which comprises:

A. providing a substantially anhydrous solution comprising the following:

a. 5-50% of tris-polyhaloalkyl phosphate containing 6 to 24 carbon atoms, and a halogen atom/carbon atom ratio of at least 0.5,

b. 2-20% nitrogenous film forming binder resin,

c. 20-80% organic solvent having a boiling point below about 200°C,

d. 0.1-5% organic aminoplast cross-linking catalyst soluble in said organic solvent;

B. impregnating cellulosic textile material with said anhydrous solution to provide therein between about 5 to 50% by weight of said phosphate based upon the dry weight of said textile material;

C. removing organic solvent from the textile material resulting from step B;

D. thereafter steaming the impregnated textile material to create therein a moisture regain in the cellulosic portion of the fabric of between about 8 and 15%; and

E. heating the textile material resulting from step (D) at a temperature between about 120° and 200°C for between about 1 to 30 minutes.

2. The process of claim 1 wherein said resin is selected from the group consisting of methoxy methyl melamine and butoxy methyl benzo quanamine.

3. The process of claim 2 wherein said phosphate is tris-(2,3-dibromopropyl) phosphate.

4. The process of claim 1 wherein said organic solvent comprises at least 90% of a haloalkane or haloalkene containing 1 to 6 carbon atoms.

5. The process of claim 1 wherein said catalyst is selected from the group consisting of haloaryllactones, haloimides and aryl sulfonyl halides.

6. The process of claim 1 wherein said catalyst is a monocyclic aryl sulfonyl chloride.

7. The process of claim 1 wherein said catalyst is p-toluene sulfonyl chloride.

8. The process of claim 1 wherein step B is performed by immersing the textile material in a bath of said mixture and then it is pad-squeezed to a wet pickup of between about 50 and 150% of said solution based on the dry weight of the textile material.

9. Fire retardant textile material produced by the process of claim 1.

\* \* \* \* \*

UNITED STATES PATENT OFFICE  
CERTIFICATE OF CORRECTION

Patent No. 3,859,124 Dated January 7, 1975

Inventor(s) James M. Thompson

It is certified that error appears in the above-identified patent and that said Letters Patent are hereby corrected as shown below:

Column 6, line 45, "Example 7" should read  
--Example 8--;

Column 8, line 39, "will" should be --with--;

Column 9, line 4, "wherein" should be --whether--;

Column 9, line 48, insert --Claims--;

Signed and sealed this 15th day of April 1975.

(SEAL)

Attest:

RUTH C. MASON  
Attesting Officer

C. MARSHALL DANN  
Commissioner of Patents  
and Trademarks